

1

2,865,751

**1-ALKYL-3-ACYLAМИDO-5-PYRAZOLONE COUPLERS FOR COLOR PHOTOGRAPHY**

George Feniak, Anthony Loria, and Warren A. Reckhow, Rochester, N. Y., assignors to Eastman Kodak Company, Rochester, N. Y., a corporation of New Jersey

No Drawing. Application September 18, 1956  
Serial No. 610,639

**4 Claims. (Cl. 96—94)**

This invention relates to 1-alkyl-3-acylamido-5-pyrazolone couplers for color photography and more particularly to such couplers in which the 3-acylamido group is a 3-phenoxyacylamido group and which substituents in the 1 and 3-positions of the pyrazolone nucleus confer special properties upon the coupler compounds.

3-acylamido-5-pyrazolone couplers for color photography have previously been described including a limited number of 1-alkyl-3-acylamido-5-pyrazolones. However, the pyrazolone coupler compounds of the present invention are distinguished in containing a particular combination of alkyl and acylamido radicals in the 1 and 3-positions of the pyrazolone nucleus with the result that dyes obtained from the couplers in the color development pro-

cess of color photography have a somewhat wider range of light absorption than do dyes prepared in a similar manner from the previously known 1-alkyl-3-acylamido-5-pyrazolones. This property of the couplers of the invention particularly adapts the couplers to use with certain benzoylacet-o-alkoxyanilide yellow dye-forming couplers in multilayer films for color photography as will be explained in more detail hereinafter.

The pyrazolone couplers of the invention have the following general structure:



wherein R represents an alkyl group of from 1 to 12 carbon atoms, R' represents a monocyclic aryl group of the benzene series such as phenyl and substituted phenyl, for example, 2,4-di-tert.-amylphenyl, 2,4-di-n-amylphenyl, n represents a positive integer of from 1 to 2, and n' represents a positive integer of from 1 to 3, R'' represents a hydrogen atom or lower alkyl group and m represents a positive integer from 1 to 2.

Representative couplers of the invention having the above general structure are as follows:

No. 1  $\lambda$  max. 520



1-methyl-3-[ $\alpha$ -(4-[ $\alpha$ -(2,4-di-tert.-amylphenoxy)butyramido]phenoxy)acetamido]-5-pyrazolone

No. 2  $\lambda$  max. 520



1-methyl-3-[ $\alpha$ -(4-[ $\alpha$ -(2,4-di-tert.-amylphenoxy)acetamido]phenoxy)acetamido]-5-pyrazolone

No. 3  $\lambda$  max. 524



1-methyl-3-[ $\gamma$ -(4-[ $\alpha$ -(2,4-di-tert.-amylphenoxy)acetamido]phenoxy)butyramido]-5-pyrazolone

No. 4  $\lambda$  max. 5241-dodecyl-3-[ $\alpha$ -(2,4-di-tert-amyloxy)acetamido]-5-pyrazoloneNo. 5  $\lambda$  max. 5231-hexyl-3-[ $\alpha$ -(2,4-di-n-amyloxy)acetamido]-5-pyrazoloneNo. 6  $\lambda$  max. 5221-hexyl-3-[ $\alpha$ -(p-[ $\alpha$ -(2,4-di-tert-amyloxy)acetamido]phenoxy)acetamido]-5-pyrazoloneNo. 7  $\lambda$  max. 5231-dodecyl-3-[ $\alpha$ -(2,4-di-n-amyloxy)acetamido]-5-pyrazoloneNo. 8  $\lambda$  max. 5231-dodecyl-3-[m-[ $\alpha$ -(2,4-di-n-amyloxy)acetamido]benzamido]-5-pyrazolone

The " $\lambda$  max" values indicated represent the wavelength of maximum light absorption of dyes made by oxidative coupling of each coupler with the developing agent 2-amino-5-diethylamino toluene hydrochloride.

The coupler compounds of the invention can be prepared in the following manner:

#### 1 - METHYL - 3 - ( $\alpha$ - (4 - NITROPHENOXY)ACETAMIDO) - 5 - PYRAZOLONE

1-methyl-3-amino 5-pyrazolone 3.4 g. (.03 mole) and  $\alpha$ -(nitrophenoxy) acetyl chloride 7.5 g. (.035 mole) were mixed in 100 ml. of dry acetonitrile and refluxed until the mixture set solid (about 1 hr.). The solid was broken up, 50 ml. of additional acetonitrile was added and the solid filtered and heated to 50° C. in 300 ml. of water containing 5 g. of sodium acetate. The solid was filtered, washed with cold water and dried.

Yield 8 g. of white product M. P. 213-215° C.

| Analysis | Calc. for (C <sub>12</sub> H <sub>12</sub> N <sub>4</sub> O <sub>5</sub> ), percent | Found, percent |
|----------|-------------------------------------------------------------------------------------|----------------|
| N.....   | 19.1                                                                                | 19.4           |

#### 1 - METHYL - 3 - ( $\alpha$ - (4 - AMINOPHOXY)ACETAMIDO) - 5 - PYRAZOLONE

1-methyl-3-( $\alpha$ -(4-nitrophenoxy) acetamido)-5-pyrazolone, 7 g. (.029 mole) was charged in a pressure bottle with 250 ml. of ethyl alcohol, 100 ml. of water and about 0.5 g. of nickel catalyst and the bottle shaken under 50 lbs. of hydrogen pressure for 1 hr. at 70-80° C. The mixture was filtered and the solvent evaporated under reduced pressure on a steam bath. The residue was dissolved in hot water, filtered and the filtrate cooled to 0° C. The precipitate which formed was filtered, washed with 20 ml. of ice water and air dried.

Yield 4.1 g. of white plates M. P. 100-102° C.

| Analysis | Calc. for (C <sub>12</sub> H <sub>14</sub> N <sub>4</sub> O <sub>5</sub> ), percent | Found, percent |
|----------|-------------------------------------------------------------------------------------|----------------|
| N.....   | 21.4                                                                                | 21.6           |

#### Coupler No. 1

1-methyl-3-[ $\alpha$ -(4-aminophenoxy) acetamido]-5-pyrazolone 2 g. (.0076 mole) and  $\alpha$ -(2,4-di-tert-amyloxy) butyryl chloride 5 g. (.015 mole) were mixed in 50 ml. of dry acetonitrile and 2 ml. of pyridine were added. After stirring the mixture for 30 min., the gum which had separated out was brought back in solution by the addition of 2 g. of KOH and 50 ml. of ethyl alcohol. After 15 min. the solution was acidified with acetic acid and the precipitate which formed on adding water (50 ml.) was filtered, washed with water and dried.

The product was obtained from petroleum ether as a white powder. Yield 2.5 g. M. P. 78-80° C.

| Analysis | Calc. for (C <sub>22</sub> H <sub>24</sub> N <sub>4</sub> O <sub>5</sub> ), percent | Found, percent |
|----------|-------------------------------------------------------------------------------------|----------------|
| C.....   | 68.1                                                                                | 68.5           |
| H.....   | 7.8                                                                                 | 7.9            |
| N.....   | 9.9                                                                                 | 9.6            |

#### Coupler No. 2

This compound was prepared as given above for coupler No. 1 except that  $\alpha$ -(2,4-di-tert-amyloxy) acetyl chloride was used instead of the  $\alpha$ -(2,4-di-tert-amyloxy) butyryl chloride.

The product was crystallized from ethyl alcohol M. P. 221-3° C.

| Analysis | Calc. for (C <sub>20</sub> H <sub>22</sub> N <sub>4</sub> O <sub>5</sub> ), percent | Found, percent |
|----------|-------------------------------------------------------------------------------------|----------------|
| C.....   | 67.2                                                                                | 67.3           |
| H.....   | 7.5                                                                                 | 7.5            |
| N.....   | 10.4                                                                                | 10.1           |

#### Coupler No. 3

A mixture of the sodium salt of p-nitrophenol (322 g.),  $\gamma$ -chlorobutyronitrile (207 g.), n-propanol (3 l.) and water (1 l.) was refluxed for 65 hours. The mixture was distilled until 2 liters of distillate was collected and the residue was poured into water (4 l.). The solid was filtered off, washed well with water and recrystallized twice from ethyl alcohol. It melted at 53-4° C. This material was hydrolyzed to  $\gamma$ -(p-nitrophenoxy) butyric acid by heating it with a 3 to 1 mixture of glacial acetic

acid and concentrated hydrochloric acid overnight on a steam bath. When the reaction mixture was cooled, the product crystallized (M. P. 127-8° C.). This acid was converted to the acid chloride with thionyl chloride under the usual conditions. The acid chloride melted at 56-7° C.

$\gamma$ -(p-nitrophenoxy) butyryl chloride (4.1 g.), which was prepared above, was added to a refluxing solution of 1-methyl-3-amino-5-pyrazolone (2.5 g.) in dry acetonitrile (100 ml.). After 5 minutes, pyridine (2 ml.) was added and the refluxing was continued for an additional 30 minutes. The reaction mixture was drowned out in water. The resulting solid was filtered off, washed with water, dried and recrystallized from absolute ethanol. It melted at 198-203° C. This material was reduced over Raney nickel in absolute ethanol at 50° C. with hydrogen at a pressure of 20 lbs. per sq. in. The ethanolic solution of 1-methyl-3-[ $\gamma$ -(p-aminophenoxy) butyramido]-5-pyrazolone thus obtained was concentrated to dryness and the residue was recrystallized from water (M. P. 140-2° C.). The product was condensed with 2 equivalents of 2,4-di-tert.-amylphenoxyacetal chloride in the presence of 2 equivalents of pyridine in dry acetonitrile at 30° C. for 30 minutes. The reaction mixture was drowned out in water and the diacyl compound was hydrolyzed with 2 equivalents of alcoholic potassium hydroxide at room temperature for 30 minutes. When the reaction mixture was acidified with acetic acid, the product separated as an oil. This was washed with water, warmed with ether, filtered and recrystallized from benzene. It melted at 135-7° C. Anal. calcd. for  $C_{32}H_{44}N_4O_5$ : C, 68.1; H, 7.8; N, 9.9. Found: C, 68.3; H, 7.9; N, 10.0.

#### Coupler No. 4

A mixture of 1-chlorododecane (400 g.), ethyl alcohol (1840 ml.) and 95% aqueous hydrazine (340 g.) was heated to reflux for 18 hours. The ethanol was distilled off under reduced pressure (20 mm.) and the residue was extracted with ether (3 l.). The ether extracts were dried and distilled. The fraction distilling at 154-8° C. at 1 mm. pressure was collected. A mixture of the dodecyl hydrazine (184 g.) obtained above, ethyl  $\beta$ -ethoxy- $\beta$ -amino-acrylate (160 g.) and absolute ethanol (920 g.) was allowed to stand at room temperature for 5 hours, then heated to reflux for 30 minutes and cooled to 0° C. The 1-dodecyl-3-amino-5-pyrazolone was filtered off and recrystallized twice from absolute ethanol. It melted at 77.5-78.5° C. This material was treated with 2 equivalents of 2,4-di-tert.-amylphenoxyacetyl chloride and 2 equivalents of N,N-dimethylaniline in refluxing acetonitrile for 3½ hours. The reaction mixture was drowned out in water. The diacylated compound was hydrolyzed with 2 equivalents of sodium hydroxide in aqueous ethanol at room temperature for 30 minutes. The reaction mixture was acidified with acetic acid, the solid product was filtered off, recrystallized from ethanol and then benzene (M. P. 78-80° C.). Anal. calcd. for  $C_{33}H_{55}N_3O_3$ : C, 73.1; H, 10.2; N, 7.8. Found: C, 73.5; H, 10.3; N, 8.1.

#### Coupler No. 5

Hexylhydrazine was converted to 1-hexyl-3-amino-5-pyrazolone (M. P. 59-62° C.) by the same procedure as was used for the conversion of dodecyl hydrazine to 1-dodecyl-3-amino-5-pyrazolone in the preparation of coupler 4. This was treated with one equivalent of 2,4-di-n-amylphenoxy acetyl chloride in refluxing acetonitrile for 45 minutes. The reaction mixture was drowned out in water and the product was recrystallized twice from methanol. It melted at 75-76.5° C. Anal. calcd. for  $C_{29}H_{33}N_3O_3$ : C, 70.8; H, 9.5; N, 9.2. Found: C, 70.8; H, 9.1; N, 9.5.

#### Coupler No. 6

Coupler 6 was prepared in the same manner as was coupler 2 except that 1-hexyl-3-amino-5-pyrazolone was used in place of 1-methyl-3-amino-5-pyrazolone. It

5 melted at 166-7° C. Anal. calcd. for  $C_{35}H_{40}N_4O_5$ : C, 69.2; H, 8.3; N, 9.2. Found: C, 69.3; H, 8.5; N, 9.2.

#### Coupler No. 7

Coupler 7 was prepared in the same manner as was coupler 4 except that 2,4-di-n-amylphenoxyacetyl chloride was used in place of 2,4-di-tert.-amylphenoxyacetylchloride. It melted at 59-61° C. Anal. calcd. for  $C_{33}H_{55}N_3O_3$ : C, 73.1; H, 10.2; N, 7.8. Found: C, 73.4; H, 10.1; N, 7.7.

#### Coupler No. 8

Coupler 8 was prepared by the procedure used for the preparation of coupler 4 except that m-[ $\alpha$ -(2,4-di-n-amylphenoxy) acetamido] benzoyl chloride was used in place of 2,4-di-tert.-amylphenoxyacetylchloride. It melted at 116.5-118° C. Anal. calcd. for  $C_{40}H_{60}N_4O_4$ : C, 72.7; H, 9.2; N, 8.5. Found: C, 72.3; H, 8.8; N, 8.7. m-[ $\alpha$ -(2,4-di-n-amylphenoxy)acetamido] benzoyl chloride, which was used above, was prepared by acylating m-aminobenzoic acid with 2,4-di-n-amylphenoxy acetyl chloride in the presence of quinoline in dioxane and converting the resulting acid to the acid chloride with thionyl chloride in the usual manner.

The benzoylacet-o-alkoxyanilide couplers with which the couplers of the present invention are particularly useful are described in the McCrossen et al., U. S. patent application Serial No. 575,099, filed March 30, 1956, and have the following general formula:



wherein R represents an alkyl group of from 1 to 30 carbon atoms and one of the groups X and Y represents a hydrogen atom and the other represents an acylamido group.

A particular group of these benzoylacet-o-alkoxyanilide couplers efficacious for use with the above couplers of the invention have the above general formula: wherein R represents an alkyl group of from about 1 to 20 carbon atoms and one of the groups X and Y represents a hydrogen atom and the other represents the group



wherein R' represents either a hydrogen atom or an alkyl group of from about 1 to 4 carbon atoms.

- 55  $\alpha$  - {3 - [ $\alpha$  - (2,4 - di - n - amylphenoxy)butyramido] - benzoyl} - 2 - methoxyacetanilide  
 3 - benzoylacetamino - 4 - methoxy - (2',4' - di - tert. - amylphenoxy) - acetanilide  
 60  $\alpha$  - {3 - [ $\alpha$  - (2,4 - di - tert. - amylphenoxy)acetamido] - benzoyl} - 2 - methoxyacetanilide  
 $\alpha$  - {3 - [ $\alpha$  - (2,4 - di - tert. - amylphenoxy)butyramido] - benzoyl} - 2 - methoxyacetanilide  
 65  $\alpha$  - benzoyl - 5 - [ $\alpha$  - (2,4 - di - tert. - amylphenoxy)butyramido] - 2 - methoxyacetanilide  
 $\alpha$  - {4 - [ $\alpha$  - (2,4 - di - tert. - amylphenoxy)acetamido] - benzoyl} - 2 - methoxyacetanilide

70 The couplers of the invention are particularly useful because the absorption maxima of the lemon-yellow dyes obtained from the latter are shifted somewhat toward the shorter wavelength of the spectrum, the absorption maxima being at about 445 millimicrons, resulting in an appreciable gap in absorption between the yellow dye and

the usual magenta dyes obtained in color development. As mentioned, the absorption maxima of typical dyes obtained from couplers No. 1 to 8 coupled with 2-amino-5-diethylaminotoluene hydrochloride in the color development reaction are given above opposite each structural formula. Therefore, since the couplers of the present invention have a somewhat broader absorption and the absorption maxima are at wavelengths in the range of 515-524 millimicrons, the gap in absorption is materially closed and the color films containing the two types of couplers more faithfully reproduce scenes in natural color.

The coupler compounds of the invention find usage in a wide variety of photographic color processes particularly wherein the couplers are dispersed in an emulsion layer such as a gelatino silver halide emulsion layer by means of coupler solvents including cellulose esters, natural and synthetic resins and organic crystallloid materials having a boiling point above about 170° C., as described in the Mannes et al. U. S. Patent 2,304,940, granted December 15, 1942, and the Jelley et al. U. S. Patent 2,322,027, granted June 15, 1943. The optimum quantity of coupler to use in the emulsion layer can be determined by simple experiment and will depend somewhat upon the coupling activity of the particular coupler, the silver halide content of the emulsion layer, the particular process in which the emulsion is to be used and other factors well known in the art of emulsion making.

In multilayer color films wherein the couplers of the invention are particularly useful, the couplers are preferably present in a green-sensitive emulsion layer and the mentioned benzoylacet-o-alkoxyanilide couplers may be present in the overlying blue-sensitive emulsion layer, a yellow filter layer intervening. A cyan coupler may then be present in the lower red-sensitive emulsion layer adjacent to the green-sensitive emulsion layer.

After exposure of the multilayer color films containing the couplers of the invention, development may be carried out by the usual methods either to obtain a color negative directly or color development may be carried out indirectly by reversal methods to obtain a color positive. A suitable color developing solution for this purpose is as follows:

|                                   | Grams |
|-----------------------------------|-------|
| 2-amino-5-diethylaminotoluene HCl | 2     |
| Sodium sulfite (anhydrous)        | 2     |
| Sodium carbonate (anhydrous)      | 20    |
| Potassium bromide                 | 1     |
| Water to 1 liter.                 |       |

In the development of exposed photographic silver halide emulsion layers, using the couplers of our invention, any color forming developer containing a primary amino group may be used. These include developers having two primary amino groups as well as those having one of the amino groups substituted or having substituents in the ring such as alkyl phenylenediamines and alkyl tolulylene diamines. These compounds are usually used in the salt form such as the hydrochloride or the sulfate which are more stable than the amines themselves. Suitable compounds are diethyl-p-phenylenediamine hydrochloride, monomethyl-p-phenylenediamine hydrochloride, dimethyl-p-phenylenediamine hydrochloride and 2-amino-5-diethylaminotoluene hydrochloride. The p-amino phenols and their substitution products may also be used where the amino group is unsubstituted. All of these developers have an unsubstituted amino group which enables the oxidation products of the developer to couple with the color forming compounds to form a dye image. The N-alkylsulfonamido alkyl-p-phenylenediamines of U. S. Patent 2,193,015 are particularly useful as color-forming developing agents.

The development process may be employed for the production of colored photographic images in layers of gelatin or other carriers, such as collodion, organic esters of cellulose, or synthetic resins. The carrier may be supported by a transparent medium such as glass, a cellulose

ester or a nontransparent reflecting medium such as paper or an opaque cellulose ester. The emulsion may be coated as a single layer on the support or as superposed layers on one or both sides of the support.

The silver halide component of the emulsion layers is not especially critical and may be, for example, silver bromoiodide, silver bromide or silver chloride, etc., depending upon the results desired. Likewise, the emulsions which are developed in the presence of the novel couplers may consist of single-layer or differentially sensitized multilayer films.

The examples and compounds set forth in the present specification are illustrative only and it is to be taken as limited only by the scope of the appended claims.

What we claim is:

1. A photographic silver halide emulsion containing a coupler compound having the general structure



wherein R represents an alkyl group of from 1 to 12 carbon atoms, R' represents a monocyclic aryl group of the benzene series, n represents a positive integer of from 1 to 2, n' represents a positive integer of from 1 to 3, R'' represents a member of the class consisting of a hydrogen atom and a lower alkyl group and m represents a positive integer from 1 to 2.

2. A photographic silver halide emulsion containing a coupler compound of the class consisting of 1 - methyl - 3 - [ $\alpha$  - {4 - [ $\alpha$  - (2,4 - di - tert - amylphenoxy)butyramido]phenoxy}acetamido] - 5 - pyrazolone; 1 - methyl - 3 - [ $\alpha$  - {4 - [ $\alpha$  - (2,4 - di - tert - amylphenoxy)acetamido]phenoxy}acetamido] - 5 - pyrazolone; 1 - methyl - 3 - [ $\gamma$  - {4 - [ $\alpha$  - (2,4 - di - tert - amylphenoxy)acetamido] - phenoxy} butyramido] - 5 - pyrazolone; 1 - dodecyl - 3 - [ $\alpha$  - (2,4 - di - tert - amylphenoxy) acetamido] - 5 - pyrazolone; 1 - hexyl - 3 - [ $\alpha$  - (2,4 - di - n - amylphenoxy)acetamido] - 5 - pyrazolone; 1 - hexyl - 3 - [ $\alpha$  - {p - [ $\alpha$  - (2,4 - di - tert - amylphenoxy) acetamido] - phenoxy}acetamido] - 5 - pyrazolone; 1 - dodecyl - 3 - [ $\alpha$  - (2,4 - di - n - amylphenoxy)acetamido] - 5 - pyrazolone; and 1 - dodecyl - 3 - {m - [ $\alpha$  - (2,4 - di - n - amylphenoxy)acetamido] - benzamido} - 5 - pyrazolone.

3. A multilayer color film comprising a support having thereon the silver halide emulsion layer of claim 1 sensitive to green light and a silver halide emulsion layer sensitive to blue light containing a coupler compound having the general formula



60 wherein R represents an alkyl group of from 1 to 20 carbon atoms and one of the groups X and Y represents a hydrogen atom and the other represents an organic acid acylamido group.

4. A multilayer color film comprising a support having thereon the silver halide emulsion layer of claim 1 sensitive to green light and a silver halide emulsion sensitive to blue light containing a coupler compound having the general formula



75 wherein R represents an alkyl group of from 1 to 20 car-

bon atoms and one of the groups X and Y represents a hydrogen atom and the other represents the group



wherein R' represents a member of the class consisting of a hydrogen atom and an alkyl group of from 1 to 4 carbon atoms.

## References Cited in the file of this patent

## UNITED STATES PATENTS

|   |           |                          |               |
|---|-----------|--------------------------|---------------|
| 5 | 2,511,231 | Weissberger et al. ----- | June 13, 1950 |
|   | 2,600,788 | Loria et al. -----       | June 17, 1952 |
|   | 2,721,798 | Loria et al. -----       | Oct. 25, 1955 |

1,070,244

## FOREIGN PATENTS

France ----- Feb. 17, 1954